

J. C. SCHMIDT.  
Whip-Handle.

No. 227,391.

Patented May 11, 1880.



Witnesses  
Wm H Chapin  
H A Chapin

Inventor  
John C Schmidt  
By Chapin & Co  
Atty's

# UNITED STATES PATENT OFFICE.

JOHN C. SCHMIDT, OF WESTFIELD, MASSACHUSETTS.

## WHIP-HANDLE.

SPECIFICATION forming part of Letters Patent No. 227,391, dated May 11, 1880.

Application filed April 28, 1879.

*To all whom it may concern:*

Be it known that I, JOHN C. SCHMIDT, of Westfield, county of Hampden, and State of Massachusetts, have invented new and useful 5 Improvements in Finishing Whip-Handles, which improvements are fully set forth in the annexed specification, and in the accompanying drawing.

The object of my invention is to provide an 10 improved finish for the handle of a plaited whip-stock; and it consists in covering the plaiting on the handle of the whip with an enamel finish, in imitation of ivory, ebony, hard rubber, or other materials, and subsequently trimming the handle in any suitable 15 way to produce the most desirable effects.

Referring to the drawing, which represents a whip-handle, *A* is the interior rattan portion thereof. *b* is the plaited covering. *c* is 20 an enamel coating applied over the plaiting *b*. *d* is a butt-tip, and *e* is a ferrule at the upper end of the enameled coating *c*.

The construction of the whip-stock as herein shown—that is, with an interior of rattan 25 pieces, *A*—is not essential for the application of my improved finish, for it is obvious that the plaiting may be braided upon any suitable material forming the stock.

After a stock has been plaited in the usual 30 manner I apply my enamel to the handle portion of the whip below the ferrule *e* and finish it thereon, producing a highly-polished surface.

For producing whip-handles in imitation of 35 ivory I apply the enamel over the plaiting and polish it, and proceed in the same manner to produce any desired color in the finish, first coloring the enamel and then applying it to the handle. After having enameled the handle I apply the butt-tip *d* and the ferrule *e* thereto, and the finish of the handle is completed.

My enamel, which consists of a mixture of

shellac, alcohol, and dry white lead, in about the proportions of one pound of shellac and 45 one pound of lead to one quart of alcohol, is a water-proof composition of considerable consistency, and when dried upon the handle is elastic and tough, and, if desired, it may be safely extended up upon the more flexible portion of the whip toward the tip without danger 50 of its becoming cracked and broken when the whip is bent.

It is obvious that the finish produced upon a whip-handle by the use of my enamel thereon 55 is much superior to that ordinarily produced from the application of a simple varnish, for while the latter does not cover the plaiting so as to form a distinct covering, my enamel does, and the plaiting is hardly, if at all, perceptible 60 upon the surface of the enamel.

By being able to produce such a perfect enameled finish upon the face of the plaited covering of a whip I am enabled to make a whip embracing the strengthening element of 65 the plaiting, no matter what may be the substance of which the stock is composed, and to produce thereupon very beautiful effects in 70 finish never yet obtained upon plaited whip handles or stocks.

What I claim as my invention is—

The hereinbefore-described improvement in 75 finishing whip-handles, which consists in applying to said handles a plaited covering, and in overlaying said plaited covering with a thick enamel capable of being finished in imitation 80 of ivory and other fancy-colored materials, and adapted to fill up the surface inequalities of said plaited covering and to provide a smooth and polished surface-finish on top of the same, substantially as set forth.

JOHN C. SCHMIDT.

In presence of—

H. A. CHAPIN,  
Wm. H. CHAPIN.